

Nov. 9, 1943.

R. JOHNSON

2,333,936

UNIFORMLY SURFACING FLAT METAL BODIES

Filed March 28, 1942

2 Sheets-Sheet 1

FIG. 1.



FIG. 2.



FIG. 3.



FIG. 4.



Inventor:

RAYMOND JOHNSON,  
by John E. Jackson  
his Attorney.

Nov. 9, 1943.

R. JOHNSON

2,333,936

UNIFORMLY SURFACING FLAT METAL BODIES

Filed March 28, 1942

2 Sheets-Sheet 2



**FIG. 6.**



**FIG. 7.**



**FIG. 8.**



**FIG. 9.**



*Inventor:*

RAYMOND JOHNSON,  
by: John E. Jackson  
his Attorney.

## UNITED STATES PATENT OFFICE

2,333,936

## UNIFORMLY SURFACING FLAT METAL BODIES

Raymond Johnson, Westmoreland County, Pa., assignor to Carnegie-Illinois Steel Corporation, a corporation of New Jersey

Application March 28, 1942, Serial No. 436,693

11 Claims. (Cl. 148—12)

The present invention relates to surfacing flat metal bodies, particularly to the disposition of uniform blue oxide finishes on steel strip and sheets.

There are many applications in the sheet metal industry in which sheet steel having a blue oxide finish is required. One of the highest requirements in this connection is that the blue oxide finish presents an absolutely uniform appearance to the eye.

Formerly the requirements of the trade were satisfied by steel sheets hot rolled on the hand mill to gauge, followed by a pickling operation. The cleaned sheets were then customarily blued in stacks by being enclosed in an annealing furnace into which steam was admitted until the desired uniformity of color was produced.

Gradually there ensued a technical transition from hot rolled products to cold rolled products, but it was found that this same practice, when applied to cold rolled sheets, did not afford the acquisition of a uniform blue oxide coating due to the inherent flatness and high surface finish of the cold rolled sheets, which caused the adjacent surfaces of the sheets in a stack intimately to engage, and thus to exclude the active oxidizing atmosphere.

It is the primary object of the present invention to teach a method for pretreating cold reduced sheets preparatory to a surface treatment thereof in stacks, such as a steam bluing operation. In a preferred embodiment of the invention, such sheets are singly passed through a corrugating or crimping device to impart a gentle undulation to the surface thereof so that when they are stacked together, the undulations do not nest but maintain the sheets in spaced relationship throughout the major portion of their surface areas. This allows for the inter-penetration of the active atmosphere during the annealing or surfacing heat treatment.

In the accompanying drawings, Figure 1 is a front view illustrating one form of crimping apparatus adapted to the practice of the present invention.

Figure 2 is a side elevational view of the apparatus shown in Figure 1.

Figure 3 is a perspective view of a stack of sheets shown in exploded relationship to illustrate the material before treatment by this method.

Figure 4 is representative of a stack of sheets after passing through the crimper.

Figure 5 is a schematic plan view, showing the manner in which the sheets are advanced into

and through the crimper preparatory to stacking.

Figure 6 represents, in plan view, one method of stacking sheets in accordance with the present invention.

Figure 7 is an elevational view of the end of the pack shown in Figure 6.

Figure 8 is a view corresponding to Figure 7 after the pack has been passed through the crimping rolls.

Figure 9 is a view similar to Figures 7 and 8 showing the sheets repacked for the steam bluing operation.

Referring more particularly to the drawings, 15 the device illustrated in Figures 1 and 2 comprises a roll stand 1 having a pair of crimping rolls 2 and 3 journaled therein in bearings 4 and 5, respectively. The lower roll 3 is arranged for revolution about a fixed axis by virtue of its bearings 5 being rigidly retained in the roll stand 1. The upper roll 2 is adapted to be raised and lowered in relation to the bottom roll, which is accomplished by its bearings 4 being vertically adjustable in the roll stand 1 by a screw-down 20 device 6 acting in opposition to a leaf spring 7 interposed between the upper bearings 4 and the lower bearings 5 of the rolls. From this arrangement it will be understood that the rolls are opened by backing-off the screw-down 6 to allow 25 the leaf spring 7 to lift the bearings 4 in relation to the bearings 5. The rolls are closed by actuating the screw-downs in an opposite direction to urge the upper bearings 4 toward the lower bearings 5 against the tension of the spring 7. 30 Any suitable arrangement is, of course, permissible to achieve this end.

The crimping rolls are preferably driven, 35 through an extension 8 of one of the necks of the lower roll 3, by a motor 9 and a reduction gear 10, which latter is connected to the roll neck extension 8 by a drive coupling 11. Suitable motor controls are conveniently placed as at 12 to vary the operating speed of the motor, thus to adjust the effective speed of the rolls to the desired 40 value.

The crimping rolls 2 and 3 are designed to 45 impart a very gradual reverse curvature to the sheets so as to avoid sharp bends or any deformation that would tend permanently to mark the sheets, since the amount of offset need be but very slight to afford optimum bluing conditions as will presently appear. It is preferred that the vertical offset of the rolls be not greater than  $\frac{1}{4}$ " from hollow to crown and the distance between crowns be sufficiently great, such as in the

order of five or six inches, to provide a very gradual curvature.

Sheet material corresponding to that shown in Figure 3 is advanced through the crimping mechanism in the manner shown in Figure 5. The sheets S are advanced through the crimping rolls, either singly or in piles, preferably in a direction agreeing with their longitudinal axes. As illustrated in this figure, they are introduced to the crimping rolls in different horizontal positions so that the corrugations or crimps resulting therefrom do not occur at the same places on each sheet in relation to the marginal portions thereof. Thus, when the sheets are finally stacked in congruent relation, as illustrated in Figure 4, the undulatory portions of the adjacent sheets are substantially opposed to afford no more than line points of contact therebetween, which allows for the inter-penetration of the active atmosphere throughout the stack, thus uniformly to coat both surfaces of each sheet irrespective of its position in the pack.

Where the sheets are passed through the crimping rolls in stacked relation, such as is desirable on gauges less than 24 gauge, a preferred arrangement for conducting this operation is shown in Figures 6 to 9 inclusive. Two or more sheets, represented in these figures S<sub>1</sub>, S<sub>2</sub>, S<sub>3</sub>, S<sub>4</sub>, and S<sub>x</sub>, are stacked with their end marginal portions in substantial alignment and with their side marginal portions relatively displaced sidewise so as to dispose the sheets in slightly offset relation, as indicated in Figures 6 and 7. Such a pack is introduced to the crimping rolls endwise so as to dispose the crimps longitudinally of the sheets. The result of this operation is illustrated in Figure 8 in which the sheets are shown in off-set nesting relationship. The sheets are then slid sideways, relative to each other until their side margins are in substantial alignment, as shown in Figure 9. This obviously disrupts the nesting relationship of the crimps and provides a pack of the desired openness.

As has been said, the extent of the offset provided by the crimping should be of a relatively slight order, preferably not to exceed  $\frac{1}{4}$ ", and for optimum results, in the order of  $\frac{1}{8}$ ". In this connection, it has been found that, where an exceedingly open pack is provided by crimps of greater magnitude, such as would be represented by commercial corrugating practice, the oxidizing action thus allowed is so severe as to build up a heavy gray oxide throughout the more exposed areas of the sheets in the pack. Such a gray oxide not only presents a non-uniform contrast to the blued areas of the more sheltered portions of the sheets, but is so brittle as to be completely cracked-off during the succeeding leveling operation so as to defeat the intended purpose. The gentle undulations or crimps, herein contemplated, afford no more than the optimum openness of pack, thus to insure of the acquisition of a uniform oxide blue coating throughout both surfaces of each sheet. It will be seen, therefore, that in addition to providing an open pack for inter-penetration of an oxidizing gas, the crimps provide a control over the extent of oxidation realized. Thus, by providing crimping rolls with an off-set deeper than is usually required, the depth of crimp imparted to any sheet, and, hence, the amount of oxidation allowed, can be varied by regulating the spacing between rolls to give any selected displacement.

In accordance with the steam bluing of the present invention, the sheets, after having been

treated as above described, are placed in an annealing receptacle and heated to the desired temperature which will be relatively high if it is desired to anneal the sheets, but which need not exceed 1000° F. if it is intended only to blue the sheets. The bluing operation is usually conducted approximately at 900° F. Thus, if the sheets have been annealed at 1200 to 1300° F., it will be necessary to allow the charge to cool to around 900° F. before introducing steam into the annealing furnace for effecting the bluing operation. Whether incident to an anneal or not, steam is introduced into the annealing container at the prescribed temperature and bathes the interior and exterior surfaces of the pack for the attainment of the blue oxide finish in a highly uniform manner.

The sheets are thereafter cooled and removed from the annealing receptacle, and may then be given one or two passes on a cold reduction mill depending on the temper and luster desired, or they may otherwise be satisfactorily treated to eliminate the crimps as on a roller leveler. There may be some applications in which it is desired to retain the crimps, in which case the material would be ready for shipment after removal from the steam blue treatment just described.

It has been stated herein that it is desired to crimp the sheets longitudinally. This is because it is customary to introduce sheets through a cold mill so that the longitudinal axis of each sheet agrees with the direction of the rolling. The desideratum here, therefore, is that the crimps extend in the direction of rolling, since they are more easily obliterated by a subsequent pass or two on a cold mill when disposed in this manner. Another reason for this practice is to dispose the crimping in that direction in which the least number of crowns are impressed into the material. By disposing the crimps longitudinally of each sheet, the number of crowns thus realized is necessarily less, by virtue of being applied across a lesser dimension of the sheet, than would be the case were they to be applied crosswise of the sheet, and, thus, extend down its greatest dimension. Any slight marking that might result from the crimping operation is, because of this, minimized by the preferred practice.

Obviously the extent of the crimping illustrated in Figure 4 has been greatly exaggerated for purposes of illustration. Actually the amount of offset provided by this crimping need be very slight in order to be effective in allowing the inter-penetration of an active atmosphere through a stack of sheets as here contemplated.

Since the apparatus and method for giving effect to the novel relationships herein disclosed may assume a variety of forms, it is intended that the herein disclosed embodiment be regarded as illustrative rather than restrictive. Therefore, it is not intended that the present invention be limited thereby other than as is necessitated by the recitation of the appended claims.

I claim:

1. The method of treating metal sheets in stacks to insure inter-penetration of the atmosphere surrounding the stack, which includes the step of plastically deforming each of the sheets throughout its cross-section so as to impart an undulatory characteristic to each sheet to disrupt the planar disposition of its surfaces, stacking said sheets so that corresponding undulations on adjacent sheets are out of registry to avoid nesting, and subjecting the stacked sheets to an active gaseous atmosphere.

2. The method of steam bluing steel sheets which includes imparting a wavy characteristic thereto preparatory to stacking, stacking such sheets in a manner to avoid nesting thereof, heating said sheets in an enclosure, and admitting steam into said enclosure to impart a blue oxide film uniformly over both surfaces of each sheet.

3. The method of steam bluing steel sheets which includes imparting a wavy characteristic thereto preparatory to stacking, stacking the wavy sheets to avoid nesting thereof, heating said sheets in an enclosure, and while heated, bathing them in steam by introducing steam into the enclosure to impart a blue oxide film to each surface of the several sheets, removing the sheets from said enclosure, and working said sheets to impart flatness, temper and luster.

4. The method of steam bluing steel sheets which includes crimping each sheet preparatory to stacking, stacking said sheets to avoid the nesting thereof, heating said sheets in an enclosure, and, while at a temperature between 800° and 1000° F., introducing steam into said enclosure to blue the sheets, removing the sheets, and working each one to flatten and impart the requisite temper and finish thereto.

5. The method of steam bluing steel sheets which includes lightly crimping a plurality of such sheets, stacking said sheets with the crimps thereof in opposition to avoid nesting, enclosing said sheets in an annealing enclosure, annealing said sheets, cooling said sheets from annealing temperature within the enclosure to a temperature between 800° to 1000° F., introducing steam into said enclosure to impart a blue oxide coloration to both surfaces of each sheet substantially uniformly, cooling said sheets to room temperature, and working said sheets to impart flatness, finish and temper.

6. The method of steam bluing steel sheets that have been cold reduced to gauge, which includes lightly crimping the cold reduced sheets preparatory to stacking, stacking several of said sheets with the corresponding crimps of adjacent sheets out of registry to provide an open pack, annealing said sheets at a temperature in the neighborhood of 1100° F., cooling the stack in the furnace down to about 900° F., introducing steam into the furnace which permeates the pack and imparts a uniform blue oxide finish to both surfaces of each sheet thereof; thereafter, cold working said blued sheets to impart the desired flatness, finish, and temper thereto.

7. In the art of bluing cold reduced steel sheets

in stacks by an oxidizing atmosphere at elevated temperature, the improvement which includes, as a preparatory step, cold straining said sheets to warp them out of a planar disposition, and stacking said sheets in non-nesting relationship to provide an open pack.

8. In the art of uniformly bluing cold reduced steel sheets in stacks by an oxidizing atmosphere incident to an annealing thereof, the improvement which includes passing each sheet through corrugating rollers lightly to corrugate it so that the corrugations fall in different places in relation to the marginal portions of each sheet, stacking the sheets in congruent relation to provide an open pack, annealing said sheets, and, while within the annealing furnace, bathing the pack in steam introduced into the furnace, cooling the sheets to room temperature, and cold working each sheet to impart flatness, finish and temper.

9. In the art of bluing cold reduced steel sheets in stacks by an oxidizing atmosphere at elevated temperature, the improvement which includes, as a preparatory step, cold straining said sheets to warp them out of a planar disposition in a recurrent offset pattern, the extent of the offset not exceeding  $\frac{1}{4}$ ", and stacking said sheets in non-nesting relationship to provide a pack of moderate openness.

10. In the art of bluing cold reduced steel sheets in stacks by an oxidizing atmosphere at elevated temperature, the improvement which includes, as a preparatory step, cold straining said sheets to crimp them in a manner to dispose the crimps so that the longitudinal axes of the latter substantially agree with the direction in which the sheet will be subsequently rolled, limiting the depth of crimp to  $\frac{1}{4}$ " or less and stacking said sheet in non-nesting relationship to provide a pack of moderate openness.

11. In the art of bluing cold reduced steel sheets in stacks by an oxidizing atmosphere at elevated temperature, the improvement which includes, as a preparatory step, stacking several sheets together with their edge portions out of substantial alignment and with their remaining portions in overlapping relationship, passing such pack endwise through crimping rolls so as to impress longitudinally extending crimps upon the pack, then re-assembling the sheets to bring their marginal portions into substantial alignment, thus to provide an open pack.

RAYMOND JOHNSON.